



US007785390B2

(12) **United States Patent**  
Johnson, Jr. et al.

(10) Patent No.: US 7,785,390 B2  
(45) Date of Patent: \*Aug. 31, 2010

- (54) **MOLYBDENUM METAL POWDER AND PRODUCTION THEREOF**

(75) Inventors: **Loyal M. Johnson, Jr.**, Tuscon, AZ (US); **Sunil Chandra Jha**, Oro Valley, AZ (US); **Carl Cox**, Tucson, AZ (US); **Patrick Ansel Thompson**, Tucson, AZ (US)

(73) Assignee: **Climax Engineered Materials, LLC**, Phoenix, AZ (US)

(\*) Notice: Subject to any disclaimer, the term of the patent is extended or adjusted under 3 U.S.C. 154(b) by 133 days.

This patent is subject to a terminal disclaimer.

(21) Appl. No.: **11/838,638**

### Prior Publication Data

US 2008/0213122 A1 Sep. 4, 2008

### Related U.S. Application Data

- (63) Continuation of application No. 10/970,456, filed on Oct. 21, 2004, now Pat. No. 7,276,102.

(51) **Int. Cl.**  
*B22F 1/00* (2006.01)  
*B22F 9/18* (2006.01)

(52) **U.S. Cl.** ..... 75/255; 75/369; 75/623

(58) **Field of Classification Search** ..... 75/255,  
75/260, 623

(56) **References Cited**

U.S. PATENT DOCUMENTS

2,398,114 A 4/1946 Rennie

- |           |   |         |                   |
|-----------|---|---------|-------------------|
| 2,402,084 | A | 6/1946  | Rennie            |
| 2,776,887 | A | 1/1957  | Kelly, Jr. et al. |
| 3,264,098 | A | 8/1966  | Heytmeijer        |
| 3,407,057 | A | 10/1968 | Timmons           |
| 3,865,573 | A | 2/1975  | Neumann et al.    |
| 3,907,546 | A | 9/1975  | Port et al.       |

(Continued)

## FOREIGN PATENT DOCUMENTS

JP 58-113369 7/1983

(Continued)

#### OTHER PUBLICATIONS

Notification of Transmittal of the International Search Report and the Written Opinion of the international Searching Authority, or the Declaration of PCT Application No. PCT/US2007/062325 mailed Aug. 4, 2008.

*Primary Examiner*—Roy King

*Assistant Examiner*—Ngoclan T Mai

(74) *Attorney, Agent, or Firm*—Fennemore Craig, P.C.

## ABSTRACT

Molybdenum metal powder has surface-area-to-mass-ratios in a range of between about 1.0 meters<sup>2</sup>/gram (m<sup>2</sup>/g) and about 3.0 m<sup>2</sup>/g, as determined by BET analysis, in combination with a particle size wherein at least 30% of the particles are larger than a size +100 standard Tyler mesh sieve. A method for producing molybdenum metal powder includes providing a supply of ammonium molybdate and a reducing gas; causing an exothermic reaction between the ammonium molybdate and the reducing gas at a first temperature to produce an intermediate reaction product and a supplemental reducing gas; causing an endothermic reaction between the intermediate reaction product and the reducing gas at a final temperature to produce the molybdenum metal powder.

## 15 Claims, 11 Drawing Sheets



## U.S. PATENT DOCUMENTS

|              |         |                     |                 |         |                  |
|--------------|---------|---------------------|-----------------|---------|------------------|
| 4,045,216 A  | 8/1977  | Meyer et al.        | 6,793,907 B1    | 9/2004  | Singh et al.     |
| 4,552,749 A  | 11/1985 | McHugh              | 6,923,842 B2    | 8/2005  | Furuya           |
| 4,595,412 A  | 6/1986  | Brunelli et al.     | 2001/0009118 A1 | 7/2001  | Hosoe et al.     |
| 4,612,162 A  | 9/1986  | Morgan et al.       | 2001/0049981 A1 | 12/2001 | McCormick        |
| 4,613,371 A  | 9/1986  | Cheney et al.       | 2003/0084754 A1 | 5/2003  | Khan et al.      |
| 4,622,068 A  | 11/1986 | Rowe et al.         | 2004/0206204 A1 | 10/2004 | Holmqvist et al. |
| 4,724,128 A  | 2/1988  | Cheresnowsky et al. | 2005/0061106 A1 | 3/2005  | Ibaraki et al.   |
| 4,915,733 A  | 4/1990  | Schiltz et al.      |                 |         |                  |
| 5,063,021 A  | 11/1991 | Anand et al.        |                 |         |                  |
| 5,330,557 A  | 7/1994  | May                 |                 |         |                  |
| 6,447,571 B1 | 9/2002  | Ito et al.          |                 |         |                  |
| 6,569,222 B2 | 5/2003  | McCormick           |                 |         |                  |
| 6,626,976 B2 | 9/2003  | Khan et al.         |                 |         |                  |

## FOREIGN PATENT DOCUMENTS

|    |             |           |
|----|-------------|-----------|
| JP | 61-201708   | 9/1986    |
| JP | 5-345903    | * 12/1993 |
| JP | 09-125101   | 5/1997    |
| JP | 2003-193152 | 7/2003    |

\* cited by examiner



FIG. 1



FIG. 2



**FIG. 3**



**FIG. 4**



**FIG. 5**



**FIG. 6**



**FIG. 7**



**FIG. 8**



**FIG. 9**



**FIG. 10**



**FIG. 11**

## 1

MOLYBDENUM METAL POWDER AND  
PRODUCTION THEREOF

## FIELD OF THE INVENTION

The invention generally pertains to molybdenum, and more specifically, to molybdenum metal powder and production thereof.

## BACKGROUND OF THE INVENTION

Molybdenum (Mo) is a silvery or platinum colored metallic chemical element that is hard, malleable, ductile, and has a high melting point, among other desirable properties. Molybdenum occurs naturally in a combined state, not in a pure form. Molybdenum ore exists naturally as molybdenite (molybdenum disulfide,  $MoS_2$ ).

Molybdenum ore may be processed by roasting to form molybdc oxide ( $MoO_3$ ), which may be further processed to form pure molybdenum (Mo) metal powder. In its pure state, molybdenum metal is tough and ductile and is characterized by moderate hardness, high thermal conductivity, high resistance to corrosion, and a low expansion coefficient. Molybdenum metal may be used for electrodes in electrically heated glass furnaces, nuclear energy applications, and for casting parts used in missiles, rockets, and aircraft. Molybdenum metal may also be used in various electrical applications that are subject to high temperatures, such as X-ray tubes, electron tubes, and electric furnaces.

## SUMMARY OF THE INVENTION

Molybdenum metal powder has surface-area-to-mass-ratios in a range of between about 1.0 meters<sup>2</sup>/gram (m<sup>2</sup>/g) and about 3.0 m<sup>2</sup>/g, as determined by BET analysis, in combination with a particle size wherein at least 30% of the particles have a particle size larger than a size +100 standard Tyler mesh sieve. Molybdenum metal powder may also be distinguished by its relatively low sintering temperature, wherein the molybdenum metal powder begins to sinter at about 950° C. The molybdenum metal powder has a final weight percent of oxygen in a range from about 0.12% to about 0.35%.

A method for producing molybdenum metal powder according to the present invention comprises providing a supply of ammonium molybdate; providing a supply of a reducing gas; causing an exothermic reaction between the ammonium molybdate and the reducing gas at a first temperature to produce an intermediate reaction product and a supplemental reducing gas; causing an endothermic reaction between the intermediate reaction product and the reducing gas at a final temperature to produce the molybdenum metal powder, the molybdenum metal powder having generally spherical particles and a surface-area-to-mass ratio between about 1.0 m<sup>2</sup>/g and about 3.0 m<sup>2</sup>/g, as determined by BET analysis.

Another embodiment of a method according to the present invention comprises providing a supply of ammonium molybdate; providing a supply of process gas; in the presence of the process gas, supplying energy to heat the ammonium molybdate at an initial temperature sufficient to decompose at least a portion of the ammonium molybdate to produce an intermediate reaction product; adjusting the energy supplied to heat the ammonium molybdate to avoid decomposing the intermediate reaction product; in the presence of process gas, supplying energy to heat the intermediate reaction product at a final temperature sufficient to reduce the intermediate reaction product; adjusting the energy supplied to heat the inter-

## 2

mediate reaction product to maintain the final temperature, the supplying energy and the adjusting energy to heat the intermediate reaction product causing formation of molybdenum metal powder, the molybdenum powder comprising generally spherical particles wherein at least 30% of the particles have a size larger than a size +100 Tyler mesh sieve.

## BRIEF DESCRIPTION OF THE DRAWINGS

10 Illustrative and presently preferred embodiments of the invention are illustrated in the drawings, in which:

FIG. 1 is a cross-sectional schematic representation of one embodiment of an apparatus for producing molybdenum metal powder according to the invention;

15 FIG. 2 is a flow chart illustrating an embodiment of a method for producing molybdenum metal powder according to the invention;

FIG. 3 is a scanning electron microscope image of the molybdenum metal powder such as may be produced according to one embodiment of the present invention wherein the ammonium molybdate precursor material is AHM;

20 FIG. 4 is a scanning electron microscope image of the molybdenum metal powder such as may be produced according to one embodiment of the present invention wherein the ammonium molybdate precursor material is AHM;

FIG. 5 is a scanning electron microscope image of the molybdenum metal powder such as may be produced according to one embodiment of the present invention wherein the ammonium molybdate precursor material is AHM;

25 FIG. 6 is a scanning electron microscope image of the molybdenum metal powder such as may be produced according to one embodiment of the present invention wherein the ammonium molybdate precursor material is ADM;

FIG. 7 is a scanning electron microscope image of the molybdenum metal powder such as may be produced according to one embodiment of the present invention wherein the ammonium molybdate precursor material is ADM;

30 FIG. 8 is a scanning electron microscope image of the molybdenum metal powder such as may be produced according to one embodiment of the present invention wherein the ammonium molybdate precursor material is ADM;

35 FIG. 9 is a scanning electron microscope image of the molybdenum metal powder such as may be produced according to one embodiment of the present invention wherein the ammonium molybdate precursor material is ADM;

40 FIG. 10 is a scanning electron microscope image of the molybdenum metal powder such as may be produced according to one embodiment of the present invention wherein the ammonium molybdate precursor material is AOM;

45 FIG. 11 is a scanning electron microscope image of the molybdenum metal powder such as may be produced according to one embodiment of the present invention wherein the ammonium molybdate precursor material is AOM.

## 55 DETAILED DESCRIPTION OF THE INVENTION

Novel molybdenum metal powder 10 has surface-area-to-mass-ratios in a range of between about 1.0 meters<sup>2</sup>/gram (m<sup>2</sup>/g) and about 3.0 m<sup>2</sup>/g, as determined by BET analysis, in combination with a particle size wherein at least 30% of the particles have a particle size larger than a size +100 standard Tyler mesh sieve. In addition, molybdenum metal powder 10 may be further distinguished by flowability in a range of between about 29 seconds/50 grams (s/50 g) and about 64 s/50 g, as determined by a Hall Flowmeter; the temperature at which sintering begins; and the weight percent of oxygen present in the final product.

Molybdenum metal powder **10** having a relatively high surface-area-to-mass-ratio in combination with a relatively large particle size and excellent flowability provides advantages in subsequent powder metallurgy processes. For example, the low Hall flowability (i.e. a very flowable material) of the molybdenum metal powder **10** produced according to the present invention is advantageous in sintering processes because the molybdenum metal powder **10** will more readily fill mold cavities. The comparatively low sintering temperature (e.g. of about 950° C.) compared to about 1500° C. for conventional molybdenum metal powders, provides additional advantages as described herein.

The novel molybdenum metal powder **10** may be produced by apparatus **12** illustrated in FIG. 1. Apparatus **12** may comprise a furnace **14** having an initial heating zone **16**, and a final heating zone **18**. Optionally, the furnace **14** may be provided with an intermediate heating zone **20** located between the initial heating zone **16** and the final heating zone **18**. A process tube **22** extends through the furnace **14** so that an ammonium molybdate precursor material **24** may be introduced into the process tube **22** and moved through the heating zones **16, 18, 20** of the furnace **14**, such as is illustrated by arrow **26** shown in FIG. 1. A process gas **28**, such as a hydrogen reducing gas **30**, may be introduced into the process tube **22**, such as is illustrated by arrow **32** shown in FIG. 1. Accordingly, the ammonium molybdate precursor material **24** is reduced to form or produce molybdenum metal powder **10**.

A method **80** (FIG. 2) for production of the molybdenum metal powder **10** is also disclosed herein. Molybdenum metal powder **10** is produced from an ammonium molybdate precursor material **24**. Examples of ammonium molybdate precursor materials **24** include ammonium heptamolybdate (AHM), ammonium dimolybdate (ADM), and ammonium octamolybdate (AOM). A method **80** for producing molybdenum metal powder **10** may comprise: i) providing **82** a supply of ammonium molybdate precursor material **24**; ii) heating **84** the ammonium molybdate precursor material **24** at an initial temperature (e.g., in initial heating zone **16** of furnace **14**) in the presence of a reducing gas **30**, such as hydrogen, to produce an intermediate product **74**; iii) heating **86** the intermediate product **74** at a final temperature (e.g., in final heating zone **18** of furnace **14**) in the presence of the reducing gas **30**; and iv) producing **88** molybdenum metal powder **10**.

Having generally described the molybdenum metal powder **10**, apparatus **12**, and methods **80** for production thereof, as well as some of the more significant features and advantages of the invention, the various embodiments of the invention will now be described in further detail.

#### Novel Forms of Molybdenum Metal Powder

Novel molybdenum metal powder **10** has surface-area-to-mass-ratios in a range of between about 1.0 meters<sup>2</sup>/gram (m<sup>2</sup>/g) and about 3.0 m<sup>2</sup>/g, as determined by BET analysis, in combination with a particle size wherein at least 30% of the particles have a particle size larger than a size +100 standard Tyler mesh sieve. In addition, molybdenum metal powder **10** may be further distinguished by flowabilities in a range of between about 29 seconds/50 grams (s/50 g) and about 64 s/50 g, as determined by a Hall Flowmeter; the temperature at which sintering begins, and the weight percent of oxygen present in the final product. As can readily be seen in FIGS. 4, 7, & 10, the combination of these unique characteristics, results in particles of novel molybdenum metal powder **10** having a generally round ball-like appearance with a very porous surface similar to that of a round sponge.

The molybdenum metal powder **10** may have surface-area-to-mass-ratios in a range of between about 1.0 meters<sup>2</sup>/gram (m<sup>2</sup>/g) and about 3.0 m<sup>2</sup>/g, as determined by BET analysis. More specifically, the molybdenum metal powder **10** may have surface-area-to-mass-ratios in the range of between about 1.32 m<sup>2</sup>/g and about 2.56 m<sup>2</sup>/g as determined by BET analysis. The high BET results are obtained even though the particle size is comparatively large (i.e. about 60 µm or 60,000 nm). Comparatively high BET results are more commonly associated with nano-particles having sizes considerably smaller than 1 µm (1,000 nm). Here, the molybdenum metal powder **10** particles are quite novel because the particles are considerably larger, having sizes of about 60 µm (60,000 nm), in combination with high BET results between about 1.32 m<sup>2</sup>/g and about 2.56 m<sup>2</sup>/g.

The molybdenum metal powder **10** particles have a particle size wherein at least 30% of the particles have a particle size larger than a size +100 standard Tyler mesh sieve. More specifically, the molybdenum metal powder **10** particles have a particle size wherein at least 40% of the particles have a particle size larger than a size +100 standard Tyler mesh sieve. Additionally, the molybdenum metal powder **10** particles have a particle size wherein at least 20% of the particles have a particle size smaller than a size -325 standard Tyler mesh sieve. Standard Tyler screen sieves with diameters of 8 inches were used to obtain the results herein.

The unique combination of high BET and larger particle size can readily be seen in FIGS. 3-11, illustrating the porous particle surface, which is similar in appearance to that of a sponge. The porous surface of the molybdenum metal powder **10** particles increases the surface-area-to-mass-ratio of the particles, providing the higher BET results. In contrast, molybdenum metal powder **10** particles that may be produced according to prior art processes have a generally smooth surface (i.e. nonporous), resulting in relatively low surface-area-to-mass-ratios (i.e. low BET results).

The relatively large particle size in combination with the approximately spherical shape of the particles contributes to low Hall flowability, making the molybdenum metal powder **10** a very flowable material and thus a good material for subsequent sintering and other powder metallurgy applications. Molybdenum metal powder **10** has flowability between about 29 s/50 g and about 64 s/50 g as determined by a Hall Flowmeter. More specifically, flowability of between about 58 s/50 g and about 63 s/50 g was determined by a Hall Flowmeter.

The molybdenum metal powder **10** may also be distinguished by its final weight percent of oxygen. Molybdenum metal powder **10** comprises a final weight percent of oxygen less than about 0.2%. Final weight percent of oxygen less than about 0.2% is a particularly low oxygen content, which is desirable for many reasons. Lower weight percent of oxygen enhances subsequent sintering processes. A higher weight percent of oxygen can often react negatively with the hydrogen gas used in the sintering furnace and produce water, or lead to higher shrinkage and or structure problems, such as vacancies. The identification of molybdenum metal powder **10** with such an advantageous weight percent of oxygen contributes to increased manufacturing efficiency.

Additionally, molybdenum metal powder **10** may be distinguished by the temperature at which sintering begins. The molybdenum metal powder **10** begins to sinter at about 950° C., which is a notably low temperature for sintering molybdenum metal. Typically, conventionally produced molybdenum metal powder does not begin to sinter until about 1500° C. The ability of the molybdenum metal powder **10** to be highly flowable and begin to sinter at such low temperatures

has significant advantages including, for example, decreasing manufacturing expenses, increasing manufacturing efficiency, and reducing shrinkage.

Molybdenum metal powder **10** may have slightly different characteristics than those specifically defined above (e.g. surface-area-to-mass-ratio, particle size, flowability, oxygen content, and sintering temperature) depending upon the ammonium molybdate precursor material **24** used to produce the molybdenum metal powder **10**. The ammonium molybdate precursor materials **24** which have been used with good results to produce molybdenum metal powder **10** include ammonium dimolybdate  $(\text{NH}_4)_2\text{Mo}_2\text{O}_7$  (ADM), ammonium heptamolybdate  $(\text{NH}_4)_6\text{Mo}_7\text{O}_{24}$  (AHM), and ammonium octamolybdate  $(\text{NH}_4)_4\text{Mo}_8\text{O}_{26}$  (AOM).

While the best results have been obtained utilizing AHM as the ammonium molybdate precursor material **24**, ADM and AOM have also been used with good results. The ammonium molybdate precursor materials **24** are produced by and commercially available from Climax Molybdenum Company in Fort Madison, Iowa.

FIGS. 3-5 are scanning electron microscope images of molybdenum metal powder **10** such as may be produced according to one embodiment of the present invention wherein the ammonium molybdate precursor material **24** was AHM. AHM is produced by and is commercially available from Climax Molybdenum Company in Fort Madison, Iowa (CAS No: 12054-85-2).

Generally, AHM may be an advantageous ammonium molybdate precursor material **24** when the final product desired must have a relatively low oxygen content and be highly flowable for applications such as sintering, for example. Using AHM as the ammonium molybdate precursor material **24** generally results in a more spherical molybdenum metal powder **10**, as shown in FIGS. 3 & 4. The spherical shape of the molybdenum metal powder **10** contributes to the high flowability (i.e. it is a very flowable material) and excellent sintering ability. The porous surface of the molybdenum metal powder **10** produced from AHM increases the surface-area-to-mass-ratio and can readily be seen in FIG. 5. Generally, molybdenum metal powder **10** produced from AHM is more flowable and has a lower oxygen content than molybdenum metal powder **10** produced from AOM or ADM.

FIGS. 6-8 are scanning electron microscope images of molybdenum metal powder **10** such as may be produced according to one embodiment of the present invention wherein the ammonium molybdate precursor material **24** was ADM. ADM is produced by and is commercially available from Climax Molybdenum Company in Fort Madison, Iowa (CAS No: 27546-07-2).

Using ADM as the ammonium molybdate precursor material **24** generally results in a more coarse molybdenum metal powder **10** than that produced from AHM, as seen in FIGS. 6 & 7. Molybdenum metal powder **10** produced from ADM also has a higher oxygen content and a lower flowability (as shown in Example 13) compared to molybdenum metal powder **10** produced from AHM. The porous surface of the molybdenum metal powder **10** produced from ADM increases the surface-area-to-mass-ratio and can readily be seen in FIG. 8. Generally, the molybdenum metal powder **10** produced from ADM has a combination of high BET (i.e. surface-area-to-mass-ratio) and larger particle size.

FIGS. 9-11 are scanning electron microscope images of molybdenum metal powder **10** such as may be produced according to one embodiment of the present invention wherein the ammonium molybdate precursor material **24** was

AOM. The AOM is produced by and is commercially available from Climax Molybdenum Company in Fort Madison, Iowa (CAS No: 12411-64-2).

Using AOM as the ammonium molybdate precursor material **24** generally results in a more coarse molybdenum metal powder **10** than that produced from AHM, as seen in FIGS. 9 & 10. Molybdenum metal powder **10** produced from AOM also has a higher oxygen content and a lower flowability (as shown in Example 14) compared to molybdenum metal powder **10** produced from AHM. The porous surface of the molybdenum metal powder **10** produced from AOM increases the surface-area-to-mass-ratio and can readily be seen in FIG. 11. Generally, the molybdenum metal powder **10** produced from AOM has a combination of high BET (i.e. surface-area-to-mass-ratio) and larger particle size.

Selection of the ammonium molybdate precursor material **24** may depend on various design considerations, including but not limited to, the desired characteristics of the final molybdenum metal powder **10** (e.g., surface-area-to-mass-ratio, size, flowability, sintering ability, sintering temperature, final weight percent of oxygen, purity, etc.).

#### Apparatus for Producing Molybdenum Metal Powder

FIG. 1 is a schematic representation of an embodiment of an apparatus **12** used for producing molybdenum metal powder **10**. This description of apparatus **12** provides the context for the description of the method **80** used to produce molybdenum metal powder **10**.

Apparatus **12** may comprise a rotating tube furnace **14** having at least an initial heating zone **16** and a final heating zone **18**. Optionally, the furnace **14** may also be provided with an intermediate heating zone **20** located between the initial heating zone **16** and the final heating zone **18**. A process tube **22** extends through the furnace **14** so that an ammonium molybdate precursor material **24** may be introduced into the process tube **22** and moved through the heating zones **16, 18, 20** of the furnace **14**, such as is illustrated by arrow **26** shown in FIG. 1. A process gas **28**, such as a hydrogen reducing gas **30**, may be introduced into the process tube **22**, such as is illustrated by arrow **32** shown in FIG. 1.

The furnace **14** preferably comprises a chamber **34** formed therein. The chamber **34** defines a number of controlled heating zones **16, 18, 20** surrounding the process tube **22** within the furnace **14**. The process tube **22** extends in approximately equal portions through each of the heating zones **16, 18, 20**. The heating zones **16, 18, 20** are defined by refractory dams **36, 38**. The furnace **14** may be maintained at the desired temperatures using any suitable temperature control apparatus (not shown). The heating elements **40, 42, 44** positioned within each of the heating zones **16, 18, 20** of the furnace **14**, provide sources of heat.

The process gas **28** may comprise a reducing gas **30** and an inert carrier gas **46**. The reducing gas **30** may be hydrogen gas, and the inert carrier gas **46** may be nitrogen gas. The reducing gas **30** and the inert carrier gas **46** may be stored in separate gas cylinders **30, 46** near the far end of the process tube **22**, as shown in FIG. 1. The process gas **28** is introduced into the process tube **22** through gas inlet **72**, and directed through the cooling zone **48** (illustrated by dashed outline in FIG. 1) and through each of the heating zones **16, 18, 20**, in a direction opposite (i.e., counter-current, as illustrated by arrow **32**) to the direction that the precursor material **24** is moved through each of the heating zones **16, 18, 20**, of the furnace **14**.

The process gas **28** may also be used to maintain a substantially constant pressure within the process tube **22**. In one embodiment of the invention, the process tube **22** may maintain water pressure at about 8.9 to 14 cm (about 3.5 to 5.5 in). The process tube **22** may be maintained at a substantially constant pressure by introducing the process gas **28** at a predetermined rate, or pressure, into the process tube **22**, and discharging any unreacted process gas **28** at a predetermined rate, or pressure, therefrom to establish the desired equilibrium pressure within the process tube **22**. The discharge gas may be bubbled through a water scrubber (not shown) to maintain the interior water pressure of the furnace **14** at approximately 11.4 cm (4.5 in).

Apparatus **12** may also comprise a transfer system **50**. The transfer system **50** may also comprise a feed system **52** for feeding the ammonium molybdate precursor material **24** into the process tube **22**, and a discharge hopper **54** at the far end of the process tube **22** for collecting the molybdenum metal powder **10** that is produced in the process tube **22**.

The process tube **22** may be rotated within the chamber **34** of the furnace **14** via the transfer system **50** having a suitable drive assembly **56**. The drive assembly **56** may be operated to rotate the process tube **22** in either a clockwise or counter-clockwise direction, as illustrated by arrow **58** in FIG. 1. The process tube **22** may be positioned at an incline **60** within the chamber **34** of the furnace **14**.

The process tube **22** may be assembled on a platform **62**, and the platform **62** may be hinged to a base **64** so that the platform **62** may pivot about an axis **66**. A lift assembly **68** may also engage the platform **62**. The lift assembly **68** may be operated to raise or lower one end of the platform **62** with respect to the base **64**. The platform **62**, and hence the process tube **22**, may be adjusted to the desired incline with respect to the grade **70**.

Although one embodiment of apparatus **12** is shown in FIG. 1 and has been described above, it is understood that other embodiments of apparatus **12** are also contemplated as being within the scope of the invention.

#### Method for Producing Molybdenum Metal Powder

A method **80** for production of the molybdenum metal powder **10** (described above) using apparatus **12** (described above) is disclosed herein and shown in FIG. 2. An embodiment of a method **80** for producing molybdenum metal powder **10** according to the present invention may be illustrated as steps in the flow chart shown in FIG. 2.

The method **80** generally begins with the ammonium molybdate precursor material **24** being introduced into the process tube **22**, and moved through the each of the heating zones **16**, **18**, **20** of the furnace **14** (while inside the process tube **22**). The process tube **22** may be rotating **58** and/or inclined **60** to facilitate movement and mixing of the ammonium molybdate precursor material **24** and the process gas **28**. The process gas **28** flows through the process tube **22** in a direction that is opposite or counter-current (shown by arrow **32**) to the direction that the ammonium molybdate precursor material **24** is moving through the process tube (shown by arrow **26**). Having briefly described a general overview of the method **80**, the method **80** will now be described in more detail.

The method begins by providing **82** a supply of an ammonium molybdate precursor material **24**. The ammonium molybdate precursor material **24** is described below in more detail. The ammonium molybdate precursor material **24** may then be introduced (i.e. fed) into the process tube **22**. The feed

rate of the ammonium molybdate precursor material **24** may be commensurate with the size of the equipment (i.e. furnace **14**) used.

As shown in FIG. 2, the method **80** continues with heating **84** the ammonium molybdate precursor material **24** at an initial temperature in the presence of the process gas **28**. As the ammonium molybdate precursor material **24** moves through the initial heating zone **16**, it is mixed with the process gas **28** and reacts therewith to form an intermediate product **74** (shown in FIG. 1). The intermediate product **74** may be a mixture of unreacted ammonium molybdate precursor material **24**, intermediate reaction products, and the molybdenum metal powder **10**. The intermediate product **74** remains in the process tube **22** and continues to react with the process gas **28** as it is moved through the heating zones **16**, **18**, **20**.

More specifically, the reaction in the initial zone **16** may be the reduction of the ammonium molybdate precursor material **24** by the reducing gas **30** (e.g., hydrogen gas) in the process gas **28** to form intermediate product **74**. The reduction reaction may also produce water vapor and/or gaseous ammonia when the reducing gas **30** is hydrogen gas. The chemical reaction occurring in initial zone **16** between the ammonium molybdate precursor material **24** and reducing gas **30** is not fully known. However, it is generally believed that the chemical reaction occurring in initial zone **16** includes the reduction or fuming-off of 60%-70% of the gaseous ammonia, reducing to hydrogen gas and nitrogen gas, resulting in more available hydrogen gas, thus requiring less fresh hydrogen gas to be pumped into the process tube **22**.

The temperature in the initial zone **16** may be maintained at a constant temperature of about 600° C. The ammonium molybdate precursor material **24** may be heated in the initial zone **16** for about 40 minutes. The temperature of the initial zone **16** may be maintained at a lower temperature than the temperatures of the intermediate **20** and final **18** zones because the reaction between the ammonium molybdate precursor material **24** and the reducing gas **30** in the initial zone **16** is an exothermic reaction. Specifically, heat is released during the reaction in the initial zone **16** and maintaining a temperature below 600° C. in the initial zone **16** helps to avoid fuming-off of molytrioxide ( $\text{MoO}_3$ ).

The intermediate zone **20** may optionally be provided as a transition zone between the initial **16** and the final **18** zones. The temperature in the intermediate zone **20** is maintained at a higher temperature than the initial zone **16**, but at a lower temperature than the final zone **18**. The temperature in the intermediate zone **20** may be maintained at a constant temperature of about 770° C. The intermediate product **74** may be heated in the intermediate zone **20** for about 40 minutes.

The intermediate zone **20** provides a transition zone between the lower temperature of the initial zone **16** and the higher temperature of the final zone **18**, providing better control of the size of the molybdenum metal power product **10**. Generally, the reaction in the intermediate zone **20** is believed to involve a reduction reaction resulting in the formation or fuming-off of water vapor, gaseous ammonia, or gaseous oxygen, when the reducing gas **30** is hydrogen gas.

The method **80** continues with heating **86** the intermediate product **74** at a final temperature in the presence of a reducing gas **30**. As the intermediate product **74** moves into the final zone **18**, it continues to be mixed with the process gas **28** (including reducing gas **30**) and reacts therewith to form the molybdenum metal powder **10**. It is believed that the reaction in the final zone **18** is a reduction reaction resulting in the

formation of solid molybdenum metal powder (Mo) **10** and, water or gaseous hydrogen and nitrogen, when the reducing gas **30** is hydrogen gas.

The reaction between the intermediate product **74** and the reducing gas **30** in the final zone **18** is an endothermic reaction resulting in the production **88** of molybdenum metal powder product **10**. Thus, the energy input of the final zone **18** may be adjusted accordingly to provide the additional heat required by the endothermic reaction in the final zone **18**. The temperature in the final zone **18** may be maintained at approximately 950° C., more specifically, at a temperature of about 946° C. to about 975° C. The intermediate product **74** may be heated in the final zone **18** for about 40 minutes.

Generally, the surface-area-to-mass-ratios (as determined by BET analysis) of the molybdenum metal powder **10** decrease with increasing final zone **18** temperatures. Generally, increasing the temperature of the final zone **18** increases agglomeration (i.e. "clumping") of the molybdenum metal powder **10** produced. While higher final zone **18** temperatures may be utilized, grinding or jet-milling of the molybdenum metal powder **10** may be necessary to break up the material for various subsequent sintering and other powder metallurgy applications.

The molybdenum metal powder **10** may also be screened to remove oversize particles from the product that may have agglomerated or "clumped" during the process. Whether the molybdenum metal powder **10** is screened will depend on design considerations such as, but not limited to, the ultimate use for the molybdenum metal powder **10**, and the purity and/or particle size of the ammonium molybdate precursor material **24**.

If the molybdenum metal powder **10** produced by the reactions described above is immediately introduced to an atmospheric environment while still hot (e.g., upon exiting final zone **18**), it may react with oxygen in the atmosphere and reoxidize. Therefore, the molybdenum metal powder **10** may be moved through an enclosed cooling zone **48** after exiting final zone **18**. The process gas **28** also flows through the cooling zone **48** so that the hot molybdenum metal powder **10** may be cooled in a reducing environment, lessening or eliminating reoxidation of the molybdenum metal powder **10** (e.g., to form MoO<sub>2</sub> and/or MoO<sub>3</sub>). Additionally, the cooling zone **48** may also be provided to cool molybdenum metal powder **10** for handling purposes.

The above reactions may occur in each of the heating zones **16**, **18**, **20**, over a total time period of about two hours. It is understood that some molybdenum metal powder **10** may be formed in the initial zone **16** and/or the intermediate zone **20**. Likewise, some unreacted ammonium molybdate precursor material **24** may be introduced into the intermediate zone **20** and/or the final zone **18**. Additionally, some reactions may still occur even in the cooling zone **46**.

Having discussed the reactions in the various portions of process tube **22** in furnace **14**, it should be noted that optimum conversions of the ammonium molybdate precursor material **24** to the molybdenum metal powder **10** were observed to occur when the process parameters were set to values in the ranges shown in Table 1 below.

TABLE 1-continued

| PARAMETER             | SETTING                       |
|-----------------------|-------------------------------|
| <u>Temperature</u>    |                               |
| Initial Zone          | about 600° C.                 |
| Intermediate Zone     | about 750° C.                 |
| Final Zone            | about 950° C.-1025° C.        |
| Time                  |                               |
| Initial Zone          | about 40 minutes              |
| Intermediate Zone     | about 40 minutes              |
| Final Zone            | about 40 minutes              |
| Process Gas Flow Rate | 60 to 120 cubic feet per hour |

As will become apparent after studying Examples 1-14 below, the process parameters outlined in Table 1 and discussed above may be altered to optimize the characteristics of the desired molybdenum metal powder **10**. Similarly, these parameters may be altered in combination with the selection of the ammonium molybdate precursor material **24** to further optimize the desired characteristics of the molybdenum metal powder **10**. The characteristics of the desired molybdenum metal powder **10** will depend on design considerations such as, but not limited to, the ultimate use for the molybdenum metal powder **10**, the purity and/or particle size of the ammonium molybdate precursor material **24**, etc.

## Examples 1 &amp; 2

In these Examples, the ammonium molybdate precursor material **24** was ammonium heptamolybdate (AHM). The particles of AHM used as the ammonium molybdate precursor material **24** in this example are produced by and are commercially available from the Climax Molybdenum Company (Fort Madison, Iowa).

The following equipment was used for these examples: a loss-in-weight feed system **52** available from Brabender as model no. H31-FW33/50, commercially available from C.W. Brabender Instruments, Inc. (South Hackensack, N.J.); and a rotating tube furnace **14** available from Harper International Corporation as model no. HOU-6D60-RTA-28-F (Lancaster, N.Y.). The rotating tube furnace **14** comprised independently controlled 50.8 cm (20 in) long heating zones **16**, **18**, **20** with a 305 cm (120 in) HT alloy tube **22** extending through each of the heating zones **16**, **18**, **20** thereof. Accordingly a total of 152 cm (60 in) of heating and 152 cm (60 in) of cooling were provided in this Example.

In these Examples, the ammonium molybdate precursor material **24** was fed, using the loss-in-weight feed system **52**, into the process tube **22** of the rotating tube furnace **14**. The process tube **22** was rotated **58** and inclined **60** (as specified in Table 2, below) to facilitate movement of the precursor material **24** through the rotating tube furnace **14**, and to facilitate mixing of the precursor material **24** with a process gas **28**. The process gas **28** was introduced through the process tube **22** in a direction opposite or counter-current **32** to the direction that the precursor material **24** was moving through the process tube **22**. In these Examples, the process gas **28** comprised hydrogen gas as the reducing gas **30**, and nitrogen gas as the inert carrier gas **46**. The discharge gas was bubbled through a water scrubber (not shown) to maintain the interior of the furnace **14** at approximately 11.4 cm (4.5 in) of water pressure.

The rotating tube furnace **14** parameters were set to the values shown in Table 2 below.

TABLE 1

| PARAMETER                  | SETTING                    |
|----------------------------|----------------------------|
| Process Tube Incline       | 0.25%                      |
| Process Tube Rotation Rate | 3.0 revolutions per minute |

TABLE 2

| PARAMETER              | SETTING                    |
|------------------------|----------------------------|
| Precursor Feed Rate    | 5 to 7 grams per minute    |
| Process Tube Incline   | 0.25%                      |
| Process Tube Rotation  | 3.0 revolutions per minute |
| Temperature Set Points |                            |
| Initial Zone           | 600° C.                    |
| Intermediate Zone      | 770° C.                    |
| Final Zone             | 946° C.-975° C.            |
| Time                   |                            |
| Initial Zone           | 40 minutes                 |
| Intermediate Zone      | 40 minutes                 |
| Final Zone             | 40 minutes                 |
| Process gas Rate       | 80 cubic feet per hour     |

Molybdenum metal powder **10** produced according to these Examples is shown in FIGS. 3-5, and discussed above with respect thereto. Specifically, the molybdenum metal powder **10** produced according to these Examples is distinguished by its surface-area-to-mass-ratio in combination with its particle size and flowability. Specifically, the molybdenum metal powder **10** produced according to these Examples has surface-area-to-mass-ratios of 2.364 m<sup>2</sup>/gm for Example 1, and 2.027 m<sup>2</sup>/gm for Example 2, as determined by BET analysis. The molybdenum metal powder **10** produced according to these Examples has flowability of 63 s/50 g for Example 1 and 58 s/50 g for Example 2. The results obtained and described above for Examples 1 and 2 are also detailed in Table 3 below.

TABLE 3

| 5  | Example/<br>Final Zone | Surface-area-<br>to-mass-ratio | Flowa-<br>bility | Final<br>Weight | Particle Size<br>Distribution by<br>Standard Sieve<br>Analysis |                      |
|----|------------------------|--------------------------------|------------------|-----------------|----------------------------------------------------------------|----------------------|
|    |                        |                                |                  |                 | Temp. (° C.)                                                   | (m <sup>2</sup> /gm) |
| 10 | 1/946° C.              | 2.364 m <sup>2</sup> /gm       | 63 s/50 g        | 0.219%          | 39.5%                                                          | 24.8%                |
|    | 2/975° C.              | 2.027 m <sup>2</sup> /gm       | 58 s/50 g        | 0.171%          | 48.9%                                                          | 17.8%                |

15 Example 1 results (listed above in Table 3) were obtained by averaging ten separate test runs. The detailed test run data for Example 1 is listed in Table 4 below. The final weight percent of oxygen in Example 1 was calculated by mathematically averaging each of the ten test runs. The surface-area-to-mass-ratio, flowability, and particle size distribution results were obtained after combining and testing the molybdenum powder products from the ten separate test runs.

20 Example 2 results (listed above in Table 3) were obtained by averaging sixteen separate test runs. The detailed test run data for Example 2 is also listed in Table 4 below. The final weight percent of oxygen in Example 2 was calculated by mathematically averaging each of the sixteen test runs. The surface-area-to-mass-ratio, flowability, and particle size distribution results were obtained after combining and testing the molybdenum powder products from the sixteen separate test runs.

TABLE 4

| Ex. # | Run # | Feed In (kg) | Feed In (g/min.) | Tube Incline % | Tube Rotation (rpm) | Initial Zone Temp. ° C. | Intermediate Zone Temp. ° C. | Final Zone Temp. ° C. | Hydrogen Gas Flow (ft <sup>3</sup> /hr) | Net Weight (kg) | Final Weight % Oxygen |
|-------|-------|--------------|------------------|----------------|---------------------|-------------------------|------------------------------|-----------------------|-----------------------------------------|-----------------|-----------------------|
| Ex. 1 | 1     | 2.415        | 8.05             | 0.25           | 3.00                | 600                     | 770                          | 946                   | 80                                      | 0.900           | 0.190                 |
|       | 2     | 1.348        | 5.62             | 0.25           | 3.00                | 600                     | 770                          | 946                   | 80                                      | 0.760           | 0.190                 |
|       | 3     | 1.494        | 6.22             | 0.25           | 3.00                | 600                     | 770                          | 946                   | 80                                      | 0.760           | 0.170                 |
|       | 4     | 1.425        | 5.94             | 0.25           | 3.00                | 600                     | 770                          | 946                   | 80                                      | 0.880           | 0.190                 |
|       | 5     | 1.689        | 7.04             | 0.25           | 3.00                | 600                     | 770                          | 946                   | 80                                      | 0.560           | 0.280                 |
|       | 6     | 2.725        | 11.35            | 0.25           | 3.00                | 600                     | 770                          | 946                   | 80                                      | 0.760           | 0.240                 |
|       | 7     | 1.492        | 6.22             | 0.25           | 3.00                | 600                     | 770                          | 946                   | 80                                      | 0.580           | 0.250                 |
|       | 8     | 0.424        | 1.77             | 0.25           | 3.00                | 600                     | 770                          | 946                   | 80                                      | 0.360           | 0.200                 |
|       | 9     | 1.752        | 7.30             | 0.25           | 3.00                | 600                     | 770                          | 946                   | 80                                      | 1.140           | 0.260                 |
|       | 10    | 0.864        | 3.60             | 0.25           | 3.00                | 600                     | 770                          | 946                   | 80                                      | 0.770           | 0.220                 |
| Ex. 2 | 11    | 0.715        | 2.98             | 0.25           | 3.00                | 600                     | 770                          | 975                   | 80                                      | 0.700           | 0.150                 |
|       | 12    | 2.575        | 10.73            | 0.25           | 3.00                | 600                     | 770                          | 975                   | 80                                      | 0.600           | 0.220                 |
|       | 13    | 1.573        | 6.55             | 0.25           | 3.00                | 600                     | 770                          | 975                   | 80                                      | 0.640           | 0.230                 |
|       | 14    | 1.376        | 5.73             | 0.25           | 3.00                | 600                     | 770                          | 975                   | 80                                      | 0.640           | 0.200                 |
|       | 15    | 1.111        | 4.62             | 0.25           | 3.00                | 600                     | 770                          | 975                   | 80                                      | 0.700           | 0.220                 |
|       | 16    | 1.53         | 6.37             | 0.25           | 3.00                | 600                     | 770                          | 975                   | 80                                      | 0.720           | 0.140                 |
|       | 17    | 1.766        | 7.36             | 0.25           | 3.00                | 600                     | 770                          | 975                   | 80                                      | 0.680           | 0.160                 |
|       | 18    | 2.038        | 8.49             | 0.25           | 3.00                | 600                     | 770                          | 975                   | 80                                      | 0.780           | 0.160                 |
|       | 19    | 1.111        | 4.63             | 0.25           | 3.00                | 600                     | 770                          | 975                   | 80                                      | 0.580           | 0.160                 |
|       | 20    | 1.46         | 6.08             | 0.25           | 3.00                | 600                     | 770                          | 975                   | 80                                      | 0.760           | 0.200                 |
|       | 21    | 1.213        | 5.05             | 0.25           | 3.00                | 600                     | 770                          | 975                   | 80                                      | 0.720           | 0.180                 |
|       | 22    | 1.443        | 6.01             | 0.25           | 3.00                | 600                     | 770                          | 975                   | 80                                      | 1.060           | 0.150                 |
|       | 23    | 1.007        | 4.20             | 0.25           | 3.00                | 600                     | 770                          | 975                   | 80                                      | 0.516           | 0.140                 |
|       | 24    | 1.848        | 7.70             | 0.25           | 3.00                | 600                     | 770                          | 975                   | 80                                      | 0.700           | 0.150                 |
|       | 25    | 1.234        | 5.14             | 0.25           | 3.00                | 600                     | 770                          | 975                   | 80                                      | 0.660           | 0.140                 |
|       | 26    | 0.444        | 1.85             | 0.25           | 3.00                | 600                     | 770                          | 975                   | 80                                      | 0.620           | 0.140                 |
| Ex. 3 | 27    | 2.789        | 11.60            | 0.25           | 3.00                | 600                     | 770                          | 950                   | 80                                      | 1.880           | 0.278                 |
|       | 28    | 4.192        | 14.00            | 0.25           | 3.00                | 600                     | 770                          | 1000                  | 80                                      | 1.340           | 0.168                 |
|       | 29    | 2.709        | 15.00            | 0.25           | 3.00                | 600                     | 770                          | 1000                  | 80                                      | 1.400           | 0.160                 |
|       | 30    | 3.21         | 13.40            | 0.25           | 3.00                | 600                     | 770                          | 1000                  | 80                                      | 1.380           | 0.170                 |
|       | 31    | 2.545        | 10.60            | 0.25           | 3.00                | 600                     | 770                          | 1000                  | 80                                      | 1.360           | 0.123                 |
| Ex. 4 | 32    | 2.617        | 10.90            | 0.25           | 3.00                | 600                     | 770                          | 1000                  | 80                                      | 1.260           | 0.117                 |

TABLE 4-continued

| Ex. # | Run # | Feed In (kg) | Feed In (g/min.) | Tube Incline % | Tube Rotation (rpm) | Initial Zone Temp. ° C. | Intermediate Zone Temp. ° C. | Final Zone Temp. ° C. | Hydrogen Gas Flow (ft <sup>3</sup> /hr) | Net Weight (kg) | Final Weight % Oxygen |
|-------|-------|--------------|------------------|----------------|---------------------|-------------------------|------------------------------|-----------------------|-----------------------------------------|-----------------|-----------------------|
| Ex. 5 | 33    | 3.672        | 15.30            | 0.25           | 3.00                | 600                     | 770                          | 1000                  | 80                                      | 1.200           | 0.173                 |
|       | 34    | 2.776        | 11.60            | 0.25           | 3.00                | 600                     | 770                          | 1025                  | 95                                      | 0.900           | 0.179                 |
|       | 35    | 2.949        | 12.30            | 0.25           | 3.00                | 600                     | 770                          | 1025                  | 95                                      | 1.720           | 0.160                 |
|       | 36    | 3.289        | 13.70            | 0.25           | 3.00                | 600                     | 770                          | 1025                  | 95                                      | 0.980           | 0.181                 |
|       | 37    | 2.329        | 9.70             | 0.25           | 3.00                | 600                     | 770                          | 1025                  | 95                                      | 1.080           | 0.049                 |
| Ex. 6 | 38    | 2.19         | 9.10             | 0.25           | 3.00                | 600                     | 770                          | 1025                  | 95                                      | 0.906           | 0.125                 |
|       | 39    | 3.187        | 13.30            | 0.25           | 3.00                | 600                     | 770                          | 950                   | 95                                      | 0.800           | 0.084                 |
|       | 40    | 3.048        | 12.70            | 0.25           | 3.00                | 600                     | 770                          | 950                   | 95                                      | 0.676           | 0.203                 |
|       | 41    | 2.503        | 10.40            | 0.25           | 3.00                | 600                     | 770                          | 950                   | 95                                      | 1.836           | 0.185                 |
|       | 42    | 2.286        | 9.40             | 0.25           | 3.00                | 600                     | 770                          | 950                   | 95                                      | 1.112           | 0.194                 |
|       | 43    | -0.01        | -0.30            | 0.25           | 3.00                | 600                     | 770                          | 950                   | 95                                      | 0.652           | 0.085                 |

## Examples 3-6

In Examples 3-6, the ammonium molybdate precursor material **24** was ammonium heptamolybdate (AHM). Examples 3-6 used the same ammonium molybdate precursor material **24**, the same equipment, and the same process parameter settings as previously described above in detail in Examples 1 and 2. Examples 3-6 varied only the temperature of the final zone. The results obtained for Examples 3-6 are shown in Table 5 below.

TABLE 5

| Example/<br>Final Zone | Surface-area-to-<br>mass-ratio | Final Weight | Particle Size<br>Distribution by<br>Standard Sieve<br>Analysis |       |
|------------------------|--------------------------------|--------------|----------------------------------------------------------------|-------|
|                        |                                |              | +100                                                           | -325  |
| Temp. (° C.)           | (m <sup>2</sup> /gm)           | % Oxygen     |                                                                |       |
| 3/950° C.              | 2.328 m <sup>2</sup> /gm       | 0.278%       | 37.1%                                                          | 21.6% |
| 4/1000° C.             | 1.442 m <sup>2</sup> /gm       | 0.152%       | 36.1%                                                          | 23.8% |
| 5/1025° C.             | 1.296 m <sup>2</sup> /gm       | 0.139%       | 33.7%                                                          | 24.2% |
| 6/950° C.              | 1.686 m <sup>2</sup> /gm       | 0.150%       | 34.6%                                                          | 27.8% |

Example 3 results (listed above in Table 5) were obtained from one separate test run. The detailed test run data for Example 3 is listed in Table 4 above. The final weight percent of oxygen, surface-area-to-mass-ratio, and particle size distribution results were obtained after testing the run data from the one test run.

Example 4 results (listed above in Table 5) were obtained by averaging six separate test runs. The detailed test run data for Example 4 is also listed in Table 4 above. The final weight percent of oxygen in Example 4 was calculated by mathematically averaging each of the six test runs. The surface-area-to-mass-ratio and particle size distribution results were obtained after combining and testing the molybdenum powder products from the six separate test runs.

Example 5 results (listed above in Table 5) were obtained by averaging five separate test runs. The detailed test run data for Example 5 is also listed in Table 4 above. The final weight percent of oxygen in Example 5 was calculated by mathematically averaging each of the five test runs. The surface-area-to-mass-ratio and particle size distribution results were obtained after combining and testing the molybdenum powder products from the five separate test runs.

Example 6 results (listed above in Table 5) were obtained by averaging five separate test runs. The detailed test run data for Example 6 is also listed in Table 4 above. The final weight percent of oxygen in Example 6 was calculated by math-

ematically averaging each of the five test runs. The surface-area-to-mass-ratio and particle size distribution results were obtained after combining and testing the molybdenum powder products from the five separate test runs.

## Examples 7-12

In Examples 7-12, the ammonium molybdate precursor material **24** was ammonium heptamolybdate (AHM). Examples 7-12 used the same ammonium molybdate precursor material **24**, the same equipment, and the same process parameter settings as previously described above in detail in Examples 1 and 2. Examples 7-12 varied in the temperatures of the intermediate and final zones. The temperatures of the intermediate and final zones and the results obtained for Examples 7-12 are shown in Table 6 below.

TABLE 6

| Example/<br>Intermediate<br>Zone Temp./<br>Final Zone | Surface-area-to-<br>mass-ratio | Flowa-<br>bility | Final<br>Weight | Particle Size<br>Distribution by<br>Standard Sieve<br>Analysis |       |
|-------------------------------------------------------|--------------------------------|------------------|-----------------|----------------------------------------------------------------|-------|
|                                                       |                                |                  |                 | +100                                                           | -325  |
| 7/ 770° C./<br>950° C.                                | 1.79 m <sup>2</sup> /gm        | 52 s/50 g        | 0.270%          | 43.8%                                                          | 16.7% |
| 8/ 760° C./<br>940° C.                                | 1.93 m <sup>2</sup> /gm        | 51 s/50 g        | 0.290%          | 51.1%                                                          | 13.7% |
| 9/ 750° C./<br>930° C.                                | 1.95 m <sup>2</sup> /gm        | 57 s/50 g        | 0.284%          | 49.5%                                                          | 14.8% |
| 10/ 740° C./<br>920° C.                               | 2.17 m <sup>2</sup> /gm        | 59 s/50 g        | 0.275%          | 43.8%                                                          | 17.2% |
| 11/ 730° C./<br>910° C.                               | 2.95 m <sup>2</sup> /gm        | 61 s/50 g        | 0.348%          | 45.6%                                                          | 16.8% |
| 12/ 770° C./<br>950° C.                               | 1.90 m <sup>2</sup> /gm        | 64 s/50 g        | 0.242%          | 50.3%                                                          | 12.5% |

Example 7 results (listed above in Table 6) were obtained by averaging nine separate test runs. The final weight percent of oxygen in Example 7 was calculated by mathematically averaging each of the nine test runs. The surface-area-to-mass-ratio, flowability, and particle size distribution results were obtained after combining and testing the molybdenum powder products from the nine separate test runs.

Example 8 results (listed above in Table 6) were obtained by averaging six separate test runs. The final weight percent

## 15

of oxygen in Example 7 was calculated by mathematically averaging each of the six test runs. The surface-area-to-mass-ratio, flowability, and particle size distribution results were obtained after combining and testing the molybdenum powder products from the six separate test runs.

Example 9 results (listed above in Table 6) were obtained by averaging eight separate test runs. The final weight percent of oxygen in Example 7 was calculated by mathematically averaging each of the eight test runs. The surface-area-to-mass-ratio, flowability, and particle size distribution results were obtained after combining and testing the molybdenum powder products from the eight separate test runs.

Example 10 results (listed above in Table 6) were obtained by averaging seventeen separate test runs. The final weight percent of oxygen in Example 7 was calculated by mathematically averaging each of the seventeen test runs. The surface-area-to-mass-ratio, flowability, and particle size distribution results were obtained after combining and testing the molybdenum powder products from the seventeen separate test runs.

Example 11 results (listed above in Table 6) were obtained by averaging six separate test runs. The final weight percent of oxygen in Example 7 was calculated by mathematically averaging each of the six test runs. The surface-area-to-mass-ratio, flowability, and particle size distribution results were obtained after combining and testing the molybdenum powder products from the six separate test runs.

Example 12 results (listed above in Table 6) were obtained by averaging sixteen separate test runs. The final weight percent of oxygen in Example 7 was calculated by mathematically averaging each of the sixteen test runs. The surface-area-to-mass-ratio, flowability, and particle size distribution results were obtained after combining and testing the molybdenum powder products from the sixteen separate test runs.

## Example 13

In Example 13, the ammonium molybdate precursor material **24** was ammonium dimolybdate (ADM). Example 13 used the same equipment and process parameter settings as previously described above in detail in Examples 1 and 2, except that the temperature of the initial, intermediate, and final heating zones was kept at 600° C. The results obtained for Example 13 are shown in Table 7 below.

TABLE 7

| Example | (m <sup>2</sup> /gm)    | (s/50 g)  | % Oxygen | Particle Size Distribution by Standard Sieve Analysis |      |
|---------|-------------------------|-----------|----------|-------------------------------------------------------|------|
|         |                         |           |          | +100                                                  | -325 |
| 13      | 1.58 m <sup>2</sup> /gm | 78 s/50 g | 1.568%   | 52.2%                                                 | 8.9% |

Example 13 results (listed above in Table 7) were obtained by averaging four separate test runs. The final weight percent of oxygen in Example 13 was calculated by mathematically averaging each of the four test runs. The surface-area-to-mass-ratio, flowability, and particle size distribution results were obtained after combining and testing the molybdenum powder products from the four separate test runs.

## Example 14

In Example 14, the ammonium molybdate precursor material **24** was ammonium octamolybdate (AOM). Example 14

## 16

used the same equipment and process parameter settings as previously described above in detail in Examples 1 and 2, except that the temperatures of the intermediate and final heating zones were varied. In Example 14 the intermediate heating zone was set between 750° C.-800° C. and the final heating zone was set between 900° C.-1000° C. The results obtained for Example 14 are shown in Table 8 below.

TABLE 8

| Example | Surface-area-to-mass-ratio (m <sup>2</sup> /gm) | Flowability (s/50 g) | Final Weight % Oxygen | Particle Size Distribution by Standard Sieve Analysis |      |
|---------|-------------------------------------------------|----------------------|-----------------------|-------------------------------------------------------|------|
|         |                                                 |                      |                       | +100                                                  | -325 |
| 14      | 2.00 m <sup>2</sup> /gm                         | >80 s/50 g (No Flow) | 0.502%                | 61.4%                                                 | 8.6% |

Example 14 results (listed above in Table 8) were obtained by averaging eleven separate test runs. The final weight percent of oxygen in Example 14 was calculated by mathematically averaging each of the eleven test runs. The surface-area-to-mass-ratio, flowability, and particle size distribution results were obtained after combining and testing the molybdenum powder products from the eleven separate test runs.

As will be understood by those skilled in the art after reviewing the above Examples, the selection of an ammonium molybdate precursor material **24** will depend on the intended use for the molybdenum metal powder **10**. As previously discussed, the selection of the ammonium molybdate precursor material **24** may depend on various design considerations, including but not limited to, the desired characteristics of the molybdenum metal powder **10** (e.g., surface-area-to-mass-ratio, size, flowability, sintering ability, sintering temperature, final weight percent of oxygen, purity, etc.).

It is readily apparent that the molybdenum metal powder **10** discussed herein has a relatively large surface-area-to-mass-ratio in combination with large particle size. Likewise, it is apparent that apparatus **12** and methods **80** for production of molybdenum metal powder **10** discussed herein may be used to produce molybdenum metal powder **10**. Consequently, the claimed invention represents an important development in molybdenum metal powder technology.

While illustrative and presently preferred embodiments of the invention have been described in detail herein, it is to be understood that the inventive concepts may be otherwise variously embodied and employed, and that the appended claims are intended to be construed to include such variations, except as limited by the prior art.

What is claimed is:

1. A molybdenum metal powder, comprising: surface-area-to-mass ratio between about 1.0 m<sup>2</sup>/g and about 3.0 m<sup>2</sup>/g, as determined by BET analysis; and particles, wherein at least 30% of the particles have a size larger than a size +100 Tyler mesh sieve.
2. The molybdenum metal powder of claim 1 further comprising a reduced form of an ammonium molybdate precursor material.
3. The molybdenum metal powder of claim 2 wherein the molybdenum metal powder begins to sinter at about 950° C.
4. A molybdenum metal powder, comprising: surface-area-to-mass ratio between about 1.0 m<sup>2</sup>/g and about 3.0 m<sup>2</sup>/g, as determined by BET analysis; and particles, wherein at least 40% of the particles have a size larger than a size +100 Tyler mesh sieve.

**17**

5. The molybdenum metal powder of claim 4, wherein the molybdenum metal powder has a flowability of between about 51 s/50 g and about 78 s/50 g as determined by a Hall Flowmeter.

6. The molybdenum metal powder of claim 4 further comprising a reduced form of an ammonium molybdate precursor material.

7. The molybdenum metal powder of claim 4 wherein the molybdenum metal powder begins to sinter at about 950° C.

8. The molybdenum metal powder of claim 1, further comprising a final weight percent of oxygen in a range from about 0.12% to about 0.35%.

9. The molybdenum powder of claim 1, wherein the molybdenum metal powder has a flowability of between about 51 s/50 g and about 78 s/50 g as determined by a Hall Flowmeter.

10. A method for producing molybdenum metal powder, comprising:

providing a supply of ammonium molybdate;  
 providing a supply of a reducing gas;  
 causing an exothermic reaction between the ammonium molybdate and the reducing gas at a first temperature to produce an intermediate reaction product and a supplemental reducing gas;

causing an endothermic reaction between the intermediate reaction product and at least the reducing gas at a final

5

10

15

20

25

**18**

temperature to produce the molybdenum metal powder, the molybdenum metal powder having a surface-area-to-mass ratio between about 1.0 m<sup>2</sup>/g and about 3.0 m<sup>2</sup>/g, as determined by BET analysis, the molybdenum metal powder comprising particles wherein at least 30% of the particles have a size larger than a size +100 Tyler mesh sieve.

11. The method of claim 10 further comprising diminishing the supply of reducing gas based on the supplemental reducing gas produced.

12. The method of claim 10 wherein the ammonium molybdate is selected from the group consisting of ammonium dimolybdate, ammonium heptamolybdate and ammonium octamolybdate.

13. The method of claim 10 wherein the molybdenum metal powder begins to sinter at about 950° C.

14. The method of claim 10 wherein the supply of reducing gas comprises hydrogen.

15. The method of claim 10, further comprising:  
 providing a supply of inert gas; and  
 using the supply of reducing gas and the supply of inert gas to maintain a substantially constant pressure during the exothermic reaction and the endothermic reaction.

\* \* \* \* \*